

Dec. 2, 1958

G. DESTRIAU

2,863,061

X-RAY FLUOROSCOPIC DEVICE

Filed May 28, 1954

2 Sheets-Sheet 1

FIG. 1.



FIG. 2.



FIG. 4.



FIG. 3.



INVENTOR.  
GEORGES DESTRIAU

BY *John J. Kelly*  
ATTORNEY

Dec. 2, 1958

G. DESTRIAU

2,863,061

X-RAY FLUOROSCOPIC DEVICE

Filed May 28, 1954

2 Sheets-Sheet 2

FIG. 5.



FIG. 6.



FIG. 7.



FIG. 8.



INVENTOR.  
GEORGES DESTRIAU

BY   
ATTORNEY.

1

2,863,061

## X-RAY FLUOROSCOPIC DEVICE

Georges Destriau, Cauderan, France, assignor to Westinghouse Electric Corporation, East Pittsburgh, Pa., a corporation of Pennsylvania

Application May 28, 1954, Serial No. 433,185

7 Claims. (Cl. 250—80)

This invention relates to X-ray devices and, more particularly, to an X-ray device having improved luminescent response to an X-ray signal.

Heretofore it has been found that an electroluminescent cell, when irradiated with X-rays, will display a decreased brightness. This "electroextinctive effect," as it has been known in the prior art, has been published on numerous occasions, a recent publication being an article by G. Destriau in Journal of Applied Physics, vol. 25, No. 1, January 1954, page 66. Other references to this "electroextinctive effect" may be found in Journal of Applied Physics, vol. 23, No. 12, December 1952, page 1289, article by Theodore Miller, and Physical Review, vol. 92 (1953), page 1323, article by Keith W. Olsen.

Also known in the prior art is the Gudden and Pohl effect which may be described as a momentary luminescence induced by the application of an electric field across a phosphor which has been previously excited.

It is the general object of this invention to provide an X-ray device which displays improved response to an X-ray signal.

It is a further object to provide an X-ray device which operates with increased brightness.

It is another object to provide an X-ray fluoroscopic device which may be operated with decreased X-ray intensity while still obtaining a usable response, thus minimizing the hazards encountered in operating X-ray equipment.

It is still another object to provide luminescent materials which may be used in X-ray fluoroscopic devices.

The aforesaid objects of the invention, and other objects which will become apparent as the description proceeds, are achieved by providing an X-ray device and luminescent material for use in combination therewith, wherein the luminescent material is irradiated by X-rays while under the influence of an electric field.

For better understanding of the invention, reference should be had to the accompanying drawings wherein:

Fig. 1 is a block diagram illustrating a fluoroscopic apparatus constructed according to this invention;

Fig. 2 is a plan view of a fluoroscopic screen as used with the device shown in Fig. 1;

Fig. 3 is a sectional elevational view taken on the line III—III of Fig. 2;

Fig. 4 is a sectional elevational view, corresponding to Fig. 3, illustrating an alternative embodiment;

Fig. 5 is a graph of screen brightness vs. periods of X-ray excitation for the electroluminescent cells of the prior art;

Fig. 6 is a graph of screen brightness vs. periods of X-ray excitation for the X-ray device of this invention;

Fig. 7 is a graph representing the sensitization ratio vs. applied electric field for the preferred fluoroscopic screen as used with this invention;

Fig. 8 is another graph representing the sensitization ratio vs. applied electric field for the fluoroscopic screen as used with this invention.

Although the principles of the invention are broadly applicable to any application wherein phosphor material is to be irradiated by X-rays, the invention has particular application with reference to fluoroscopic screens, and hence it has been so illustrated and will be so described.

2

With particular reference to the form of the invention illustrated in the drawings, the numeral 10 in Fig. 1 indicates generally a fluoroscopic apparatus which generally comprises a fluoroscopic screen 12, electric field voltage supply 14, inspection table 16 and X-ray generating apparatus 18, which X-ray apparatus may be of 80 kv., 3 ma. rated output, for example.

In Figs. 2 and 3 are illustrated the preferred embodiment of the fluoroscopic screen 12 which comprises generally a substantially planar layer of luminescent material 20 in contact with a substantially planar layer of dielectric material 22, said luminescent material and dielectric being sandwiched between two thin transparent conducting layers or electrodes 24 and 26. A foundation-viewing plate 28 is placed over one of the conducting layers, for example layer 24, and an insulating layer 30 is placed over the other conducting layer in order to minimize shock hazard. Each of the conducting layers 24 and 26 are connected by separate electrical leads 32 and 34 to the field voltage supply 14, as shown in block diagram in Fig. 1. A protecting and handling shield 36 is normally provided around the entire periphery of the cell in order to facilitate handling, storage, etc.

The luminescent material 20 is preferably positioned next to the foundation-viewing plate 28 in order to improve screen perception and minimize parallax, although for some applications it might be preferable to place the dielectric material 22 next to the viewing plate. The luminescent material 20 will be more thoroughly considered in the following paragraphs and for such an application as the instant one may have a thickness of about 0.2 mm., although this thickness is no way critical. Where the phosphor and dielectric materials are included in separate layers, as illustrated in Fig. 3, the dielectric may consist of any material which has a high dielectric constant, is transparent to X-rays and will not deteriorate under the action of X-rays. Such materials are well known and, as an example, the dielectric material may consist of a mica sheet about 0.05 mm. thick although this thickness is in no way critical and may be increased or decreased as dictated by the application.

The thin transparent conducting electrodes 24 and 26 may be any conducting transparent materials which may readily be coated as a thin sheet, are transparent to visible light in the case of the upper layer 24 and transparent to X-rays in the case of the lower layer 26, and will not deteriorate appreciably under the action of X-rays. As an example, the coating 24 may be of tin oxide and may be applied as described in Patent No. 2,522,531 to Mochel. Alternatively the coating 24 may be of an oxide of zinc, cadmium, aluminum or bismuth. The thin transparent conducting coating 26 may be of tin oxide, or may be a thin reflecting coating of aluminum which may be applied by the well-known vacuum-metallizing techniques, a representative thickness of such Al coating being 0.001 cm. The thin protective layer 30, which is intended to insure against shock hazard and to facilitate handling, may be of any X-ray transparent material which has a relatively high dielectric constant, an example being a polystyrene compound as sold by Dow Chemical Co. under the trademark "Styron." Another example of a satisfactory material is a methyl methacrylate compound, such as sold by E. I. du Pont under the trademark "Lucite." This protective coating 30 may be dispensed with if desired as it in no way affects the operation of the device. Shock hazard may then be eliminated by grounding the electrode 26.

The foundation glass-viewing plate 28 may be fabricated of any glass which contains heavy atoms which will absorb the X-rays and thus protect the viewer. As an example, any of the well-known lead or cerium glasses

may be used. The protecting shield 36 may be of any suitable plastic material such as the aforementioned polystyrene compound. This protecting shield is in no way necessary to the operation of the device and may be dispensed with if desired.

The electrical leads 32 and 34 may be directly connected to the electrodes 24 and 26 respectively or preferably are connected to the electrodes through bus bars 38 and 40 as described in Patent No. 2,628,299 to Gaiser.

The field voltage supply may consist of a transformer having an output which is variable between 100 and 2,000 volts, 60 cycles, for example, in order that the field applied across the electrodes may be adjusted to optimum conditions, as hereinafter explained.

In Fig. 4 is represented an alternative embodiment of the fluoroscopic screen, as illustrated in Fig. 3, and all parts of this alternative embodiment are identical with the embodiment as illustrated in Fig. 3 except that the phosphor is embedded throughout the dielectric, to form a homogeneous phosphor-dielectric layer 40. In such an embodiment the dielectric in which the phosphor is embedded may consist of any material which is relatively transparent to visible light and X-rays, is stable under the action of X-rays and has a high dielectric constant, a dielectric constant about 4 being generally satisfactory. This requirement of high dielectric constant for the dielectric, however, is one of preference rather than necessity since the fields which are utilized in the instant application are relatively small as compared to the fields which are normally desirable in the usual electroluminescent cell or lamp applications where the cell brightness is dependent upon the field applied. As examples of a dielectric in which the phosphor is embedded, either of the heretofore-mentioned polystyrene or methyl methacrylate compounds will be satisfactory. An X-ray transparent glass such as a boro-silicate glass having a phosphor embedded throughout can also be used and the glass-dielectric layer may be fabricated as described in copending application of Eugene Etzel, Serial No. 419,232, filed March 29, 1954, entitled "Phosphor Embedded Glass and Method of Making." In the embodiment of the invention of Fig. 4, an equivalent amount of phosphor may be embedded in the dielectric as would form a phosphor layer about 0.2 mm. thick, as described in the preferred embodiment of Fig. 3. This amount of phosphor, however, is only one of choice and the amount may be varied as dictated by the application. Sufficient dielectric material may be incorporated with the phosphor to cause the phosphor-dielectric layer to be about 0.3 mm. thick. This thickness is given only by way of example and not by way of limitation and may be varied according to the application.

In Fig. 5 is illustrated a graph of arbitrary brightness units vs. time in minutes of X-ray irradiation for a fluoroscopic screen incorporating a known fluoroscopic phosphor and adapted to have an electric field applied thereacross. The prior art phosphor material utilized in the screen is ZnCdS:Ag of 0.2 mm. thickness, which is a well-known X-ray-sensitive phosphor. In this experiment this phosphor is placed between two electrodes, as illustrated in Fig. 3. When the fluoroscopic screen embodying this phosphor is irradiated with X-rays, the brightness increases following the curve OABC. When a field is applied between the two electrodes, simultaneously with the X-ray irradiation, the brightness may be represented by the curve OA'B'C'. If the electric field is applied only between the time  $t_1$  and  $t_2$  there is a sudden drop AD in brightness upon application of the field at  $t_1$ , after which the brightness slowly increases from its minimum at D to point B', which is the brightness normally expected with both X-ray irradiation and applied field. When the field is removed at time  $t_2$ , there is experienced a small drop B'E, after which the brightness increases to that normally expected with only X-ray irradiation.

If a ZnCdS:Mn phosphor is incorporated in the pre-

ferred embodiment of the screen, as illustrated in Fig. 3, the effect of decreased brightness, as illustrated in Fig. 6, is completely reversed and an increased brightness is obtained. There is illustrated in Fig. 6 a graph of arbitrary brightness units vs. periods of X-ray irradiation for the preferred ZnCdS:Mn phosphor incorporated into a fluoroscopic screen, as illustrated in Fig. 3. All brightness measurements referred to were made under the same test conditions and thus represent relative values.

10 One embodiment of this phosphor consists of 2 moles CdS, 7 moles ZnS and activated by  $5 \times 10^{-2}$  mole Mn. Such a phosphor may be prepared by ball-milling the aforementioned ingredients and firing in an oxygen-free atmosphere for about one hour at 1200° C. Where this aforementioned ZnCdS:Mn phosphor is incorporated into the fluoroscopic screen, an exactly opposite result is obtained than was obtained with the prior art X-ray phosphors. With reference to Fig. 6, if no field is applied and the screen is irradiated with X-rays, the brightness follows the curve PFGH. If an electric field is applied simultaneously with X-ray irradiation, the brightness follows the curve PF'G'H', which curve PF'G'H' is above the curve PFGH, contrary to the results obtained with prior art phosphors. If the screen is irradiated only with X-rays up to the time  $t_1$  and then the field is suddenly applied, there is a sudden increase in brightness from F to K. The brightness then slowly decreases to the brightness which is to be expected when both electric field excitation and X-ray irradiation are simultaneously applied. If the field is removed at  $t_2$  there is a small increase in brightness which follows the curve G'L and the brightness then decreases to that which would be normally expected were only X-ray irradiation applied to the screen. It is to be observed that just 35 the opposite results are obtained where the phosphor of this invention is used, as has been experienced where the X-ray sensitive luminescent materials of the prior art have been used in identical experiments.

As heretofore noted, a specific example of the phosphor 40 which may be used in the fluoroscopic screen consists of 2 moles CdS, 7 moles ZnS and activated by  $5 \times 10^{-2}$  mole Mn. It has been found that this luminescent material activated by from about  $0.01 \times 10^{-2}$  to  $6 \times 10^{-2}$  mole Mn per mole of zinc plus cadmium will be satisfactory and 45 apparently the main constituents of the phosphor which affect its properties regarding increased brightness when irradiated by X-rays and placed within an electric field are CdS and Mn. It has been found that the ratio of Cd to Zn in the luminescent material should be from between 1 mole CdS; 9 moles ZnS to 7 moles CdS; 3 moles ZnS, if a satisfactory output is to be obtained. Any molar ratio of Cd to Zn within these aforementioned 50 limitations will produce a luminescent material which is generally satisfactory for the disclosed fluoroscopic screens. The moles of Mn activator per mole of Cd and Zn are preferably from about  $0.3 \times 10^{-2}$  to about  $1.1 \times 10^{-2}$ , although this range may vary from 0.01 to  $10^{-2}$  to  $6 \times 10^{-2}$  mole Mn activator per mole of luminescent material, as heretofore mentioned.

In order to increase the X-ray sensitivity of the luminescent material, there may be added to the aforementioned phosphor from traces, e. g.  $0.001 \times 10^{-2}$  mole Ag up to about  $1.0 \times 10^{-2}$  mole of Ag activator per mole of Mn activator. This Ag activator addition will not measurably decrease the increase in brightness which is realized thru the screen excitation by both X-ray irradiation and an electric field, but the silver activator addition increases somewhat the X-ray sensitivity of the phosphor.

Luminescent material compositions according to this 70 invention are given in the following examples:

#### Example 1

2 moles CdS

7 moles ZnS

$5 \times 10^{-2}$  mole Mn

## 5

## Example 2

1.5 moles CdS  
5 moles ZnS  
 $2 \times 10^{-2}$  mole Mn

## Example 3

2 moles CdS  
7 moles ZnS  
 $5 \times 10^{-2}$  mole Mn  
 $0.01 \times 10^{-2}$  mole Ag

In the usual type of electroluminescent cell, which is normally constructed as a phosphor-embedded dielectric sandwiched between two electrodes, the cell brightness is directly proportional to the field intensity. In contrast, in the fluoroscopic screen used with this invention, the field intensity is at an optimum at about 15-25 kv. per cm. There is illustrated in Fig. 7 a graph of relative intensity vs. applied electric field for the phosphor as given in Example 1. As shown, the maximum phosphor relative brightness occurs at about 15 kv. per cm. and is about  $2.3 P_1$ .  $P_1$  is a sensitizing ratio and represents the brightness ( $b_1$ ) of the fluoroscopic screen when the screen is irradiated by X-rays and has simultaneously applied thereto an electric field, divided by the brightness ( $b_0$ ) of the same screen when irradiated by X-rays only. Thus  $P_1 = b_1/b_0$ .

In Fig. 8 is represented the sensitizing ratio ( $P_1$ ) vs. field in applied kv. per cm. for the phosphor given in Example 2. As illustrated, the maximum sensitizing ratio occurs at about 18 kv. per cm. and is about 1.6, after which the sensitizing ratio decreases. This phenomenon of decreasing sensitizing ratio after an optimum has been reached has been generally observed with the luminescent materials of this invention and in all experiments conducted so far the optimum field occurs between 15 and 25 kv./cm. In order to operate at the field of 20 kv./cm. for the specific example of the embodiment as illustrated in Fig. 3, wherein the combined thickness of phosphor and dielectric is 0.25 mm., the applied voltage to the electrodes should be about 500. In order to operate at about the optimum for the specific example of the alternate embodiment as given in Fig. 4 where the phosphor-dielectric is 0.3 mm. thick, the applied voltage to the electrodes should be about 600.

It will be observed that when operating a fluoroscopic apparatus, as shown in Fig. 1, when examining an iron casting, etc. the X-ray irradiation and electric field excitation may be simultaneously applied to the fluoroscopic screen which will result in a brightness far superior to that realized in prior art practices.

As an alternative method of operation, the X-ray intensity may be decreased from the X-ray intensity required to operate the fluoroscopes of the prior art, and a picture of equivalent brightness may still be obtained. This of course has the advantage of decreasing the hazards encountered in operating X-ray equipment.

It will be recognized that the objects of the invention have been achieved by providing an X-ray device which operates with increased brightness, or which device may be operated with decreased X-ray intensity and still have a brightness which is equivalent to that of the X-ray devices of the prior art. Phosphor materials for use in combination with such X-ray devices have also been provided.

While in accordance with the patent statutes one best known embodiment of the invention has been illustrated and described in detail, it is to be generally understood that the invention is not limited thereto or thereby.

I claim:

1. An X-ray sensitive device comprising, a screen comprising luminescent material sandwiched between two electrodes, means for applying an alternating current po-

## 6

tential between said electrodes, means for irradiating said luminescent material with X-rays, and said luminescent material consisting of ZnS and CdS wherein the molar ratio of Zn to Cd is from 9 Zn:1 Cd to 3 Zn:7 Cd and activated by from  $0.01 \times 10^{-2}$  to  $6.0 \times 10^{-2}$  mole Mn per mole of luminescent material.

5 2. An X-ray sensitive device comprising, a screen comprising luminescent material sandwiched between two electrodes, means for applying an alternating current potential between said electrodes, means for irradiating said luminescent material with X-rays, and said luminescent material consisting of ZnS and CdS wherein the molar ratio of Zn to Cd is from 9 Zn:1 Cd to 3 Zn:7 Cd and activated by from  $0.3 \times 10^{-2}$  to  $1.1 \times 10^{-2}$  mole Mn per mole of luminescent material.

10 3. A fluoroscopic device comprising, a luminescent material and a dielectric sandwiched between two electrodes, means for applying an alternating current potential between said electrodes, means for irradiating said luminescent material with X-rays, said luminescent material consisting of ZnS and CdS wherein the molar ratio Zn to Cd is from 9 Zn:1 Cd to 3 Zn:7 Cd and activated by one of the group consisting of Mn, and Mn and Ag, said Mn activator being present in amounts of from 20  $0.3 \times 10^{-2}$  to  $1.1 \times 10^{-2}$  mole per mole of luminescent material, and said Ag activator being present in amounts of from traces to  $1.0 \times 10^{-2}$  mole per mole of Mn activator.

15 4. An X-ray sensitive device comprising, a screen including luminescent means which exhibits the property of sustained luminescence under excitation by X-rays and sustained enhanced luminescence under the simultaneous influence of an alternating electric field, means for applying an alternating electric field across said luminescent means, and means for simultaneously irradiating said luminescent means with X-rays.

20 5. An X-ray sensitive device comprising, a screen of dielectric and luminescent means, said luminescent means exhibiting the property of sustained luminescence under excitation by X-rays and sustained enhanced luminescence under the simultaneous influence of an alternating electric field, means for applying an alternating electric field across said screen, and means for simultaneously irradiating said screen with X-rays.

25 6. An X-ray sensitive device comprising, a screen including finely-divided luminescent means which exhibits the property of sustained luminescence under excitation by X-rays and sustained enhanced luminescence under the simultaneous influence of an alternating electric field, means for applying an alternating electric field across said luminescent means, and means for simultaneously irradiating said luminescent means with X-rays.

30 7. An X-ray sensitive device comprising, a screen of dielectric and finely-divided luminescent means, said luminescent means exhibiting the property of sustained luminescence under excitation by X-rays and sustained enhanced luminescence under the simultaneous influence of an alternating electric field, means for applying an alternating electric field across said screen, and means for simultaneously irradiating said screen with X-rays.

## References Cited in the file of this patent

## UNITED STATES PATENTS

65 2,566,349 Mager ----- Sept. 4, 1951  
65 2,650,310 White ----- Aug. 25, 1953

## OTHER REFERENCES

70 Luminescent Materials, by Leverenz et al., Journal Applied Physics, July 1939, pages 487 and 488.  
Transient Voltage Indicator and Information Display Panel, Bramley et al., Review of Scientific Inst., June 1953, vol. 24, pages 471-2.